# EUROPEAN PATENT SPECIFICATION

(11) **EP 1 660 704 B1**
(45) Date of publication and mention of the grant of the patent: **15.07.2009**
(21) Application number: 03751726.5
(22) Date of filing: 02.09.2003
(51) Int. Cl.: D01D 5/00, C09D 127/12

(54) **PROCESS FOR PREPARING SUPERHYDROPHOBIC SURFACE COMPOSITIONS, SURFACES OBTAINED BY SAID PROCESS AND USE OF THEM**
VERFAHREN ZUR HERSTELLUNG VON SUPER-HYDROPHOBEN OBERFLÄCHEN, DARAUS HERGESTELLTE OBERFLÄCHEN UND DEREN VERWENDUNG
PROCEDE DE PREPARATION DE COMPOSITIONS DE SURFACE SUPERHYDROPHOBE, SURFACES OBTENUES PAR LEDIT PROCEDE ET LEUR UTILISATION

(43) Date of publication of application: 31.05.2006
(73) Proprietor: Sabanci Universitesi, 34956 Tuzla-Istambul (TR)
(72) Inventor: ACATAY, Kazim Sabancy University, 34956 Tuzla-Istanbul (TR); GULGUN, Mehmet Ali, Sabanci University, 34956 Tuzla-Istanbul (TR); MENCELOGLU, Yusuf Ziya, Sabanci University, 34956 Tuzla-Istanbul (TR)
(74) Representative: Arkan, Selda Mine
(86) International application number: PCT/TR2003/000067
(87) International publication number: WO 2005/021843

(56) References cited:
- EP-A- 0 949 296
- US-A1- 2003 013 795
- DEITZEL J M ET AL: "Electrospinning of polymer nanofibers with specific surface chemistry" POLYMER, ELSEVIER SCIENCE PUBLISHERS B.V, GB, vol. 43, no. 3, March 2002 (2002-03), pages 1025-1029, XP004323626 ISSN: 0032-3861

## Description

The present invention relates to a process for preparing super-hydrophobic surface compositions and to compositions obtained by said process. More precisely the present invention relates to an electrospinning or electrospraying process for preparing super hydrophobic surface compositions and to nanofabricated super-hydrophobic surfaces obtained by this process. The invention also relates to the use of the super-hydrophobic surfaces obtained.

The term of super-hydrophobicity is related with surface tension/energy. Surface tension/energy is an internal force due to an unbalance in molecular forces that occur when two different materials are brought into contact with each other forming an interface or boundary. At the liquid-surface interface, if the adhesive forces are stronger than the cohesive forces, the molecules of the liquid have a stronger attraction to the molecules of the solid surface than to each other and wetting of the surface occurs. If the adhesive forces are weaker, the liquid does not wet the surface of the solid.

Surface energy of a solid can be determined by Goniometry in that the contact angle of various liquids on a surface is measured. These contact angle values are related with surface energy by empirical or theoretical equations according to various theories. Water contact-angle on a solid surface larger than 140-160° represents a super-hydrophobic surface.

Generally, super-water repellent surfaces are created either by tailoring the surface chemistry and topography with various time consuming and complex techniques or by creating hydrophobic surface that is not solvent resistant.

Compositions for producing difficult to wet surfaces are given in EP-A-1.153.987. EP-A-1.238.717 relates to the geometric shaping of surfaces having a Lotus effect. EP-A-1.249.280 and EP-A-1.249.281 relate to self-cleaning surfaces with hydrophobic structures and process for making them. EP-A-1.249.467 and EP-A-1.249.468 relate to self-cleaning surfaces due to hydrophobic structure and process for the preparation thereof and EP-A-1.283.077 relates to obtaining a lotus effect by preventing microbial growth on self-cleaning surfaces.

As can be seen considerable scientific and industrial research activities are performed on development of super-hydrophobic, low surface energy, polymeric coating surfaces. But none of these techniques is particularly robust or long lasting, and can be controlled on a more substantial scale except in very clean environments.

It is an aim of the present invention to provide a method for making coatings in a short time and with a simple equipment requirement. It is also an aim of the present invention to provide coatings having ease and minimal cost of application. It is another aim of the present invention to provide coatings with good film forming properties having high surface area to volume ratio. It is another aim of the present invention to provide coatings with tuneable surface properties, such as hydrophobic, lypophobic, antibacterial etc. Finally it is an aim of the present invention to provide super-hydrophobic coatings.

The above aims have been achieved by Applicants invention.

The invention relates to a process for preparing super-hydrophobic surface compositions comprising the steps
a) radical or condensation polymerisation of a reactive functional group containing monomer pair with an initiator in non-reactive solvent environment, and
b) mixing the copolymer obtained in a) with a hydrocarbon/fluorinated/siloxane chemical agent having at least one end capped with reactive groups and a catalyst.
   characterised In that it further comprises the step of
c) electrospinning/ electrospraying of the mixture obtained in b), and
d) annealing and crosslinking of the electrospun/ electrosprayed mixture.

In step a) that the monomer pairs are radical or condensation polymerisable monomers and their combination and step growth polymerisable monomers where one of them contains fluoro/siloxane/hydrocarbon alkyl group and a reactive functional group chosen from the group comprising TMI/AN, TMI/Styrene, TMI/polymethylmethacrylate and perfluoro-alkyl acrylate/vinyl benzyl-dimethyl-cocoamonium chloride (VBDMCAC).

In step a) the initiator is a radical generating initiator or condensation polymerisation catalyst chosen from the group comprising azo initiators such as AIBN, peroxide initiators such as BPO, ammonium persulphate, sodium persulphate and T2EH. Again in step a) the non reactive solvent is preferably chosen from the group comprising dimethyl formamide (DMF), tetrahydro furan (THF), chloroform, methylene chloride, toluene, dichloromethane, ethanol, formic acid, dimethylacetamide, acetone.

In step b) the hydrocarbon/fluorinated/siloxane chemical agent has both ends capped with reactive groups such as hydroxyl, amine, carboxyl, isocyanate, thiol. Preferably the both end reactive group containing agent is chosen from the group comprising, (perfluoropolyether, PFPE) HOCH₂CF₂(OCF₂)ₙ(OCF₂CF₂)ₘCF₂CH₂OH, (siloxane diols) HO(Me₂Si-O)ₙH. (hydrocarbon diol) HO(CH₂)ₙOH, and (polyether diol) HO(CH₂CH₂O)ₙH.

Again in step b) the catalyst is chosen from the group containing stannous-2-ethyl hexanoate (T2EH), cobalt-2-ethyl hexanoate, dibutyltin dilaurate,etc.

In step c) a polymer solution or melt, held by surface tension at the end of a capillary, is subjected to a high electric field (Up to 20-30 kV). A jet of the solution ejected from the tip is charged and directed to a grounded collector, the solvent evaporates and a continuous, non-woven, ultra-thin (40-2000 nm in diameter) fibres and particles can be collected. Electrospraying process needs higher applied voltages and nanometer or micrometer range small, polymer solution droplets are transferred to the grounded screen.

The advantages of electro-spinning/ spraying are its ability to make fibres/ particles in the range of nanometers (one to two orders of magnitude smaller than the conventional fibres), high surface area to volume ratio, equipment requirement is simple and spinning time is much shorter than the conventional spinning.

Also, the material's bulk properties effect decreases in nanometer scale and the atomic properties becomes more effective. So, the material may show strange properties when compared with the bulk properties in nanometer diameter. By the aid of electrospinning/spraying, tunable surface properties can emerge.

The invention also relates to super-hydrophobic surface compositions obtained by the above process and to the use of these super-hydrophobic surface compositions.

Said use can be in the prevention of adhesion of dirt and foreign materials to materials like antennas, windows, bio-reactors, solar cells, traffic indicators, public transports and animal cages.

Said use can also be in antifouling applications in human made marine vessels and buildings, haven appliances and oil-drilling platforms. Also said use can be in stain resistance of the materials in saunas, swimming-pools, bathrooms, kitchens, roofs, walls, facades, green-houses, garden fences, wood appliances.

Finally said use can be in multi-functional membranes, biomedical structural elements (scaffolding used in tissue engineering, wound dressing, drug delivery, artificial organs), protective shields in specialty fabrics, filter media for submicron particles in separation industry, composite reinforcement, and structures for nano-electric machines.

The accompanying drawings, which are included to provide a further understanding of the invention and are hereby incorporated in and constitute a part of this specification, illustrate embodiments of the invention and together with the specification serve to explain the principles of the invention.

In the drawings:
- Figure 1: is the scanning electron microscope image of electrospray film at 15kV
- Figure 2: is the scanning electron microscope image of electrospray film at 10kV
- Figure 3: is the scanning electron microscope image of electrospun film at 7kV
- Figure 4: shows an enlarged image of Figure 3
- Figure 5: shows contact angle photograph of water a) on a electrospun web of mixture, b) on a cast film of same mixture and c) on a condensation route polymerised sample
- Figure 6: shows the scanning electron image of an electrospun film obtained according to Example 2
- Figure 7: shows the secanning electron image of an electrospun film obtained by fluorinated diol substitution in addition polymerisation with crosslinker route

It is to be understood that the foregoing general description and the following detailed description are exemplary and explanatory and are intended to provide further explanation of the invention as claimed.

The invention concerns an electrospinning/ electrospraying processes for preparing super-hydrophobic surface compositions and to nanofabricated super-hydrophobic surfaces obtained. The surface of the perfluorinated/siloxane/hydrocarbon and crosslinked copolymeric resins shows after electro-spinning/ spraying and annealing super hydrophobic property.

The prepared coating material can be tailored to various conditions over a wide range of amphipilicy (chemically and topographically) and those properties can be adjusted or tuned without adversely affecting the stability, curability, or mechanical properties of the material.

For obtaining super-hydrophobicity, the solid surface is enhanced chemically by using fluorine/silicone containing moieties in the material. These materials exhibit low surface energy, low water absorptivity, stain resistance, high thermal stability, higher level of chemical inertness and excellent weatherability

Another point for chemical enhancement is segregation of fluorinated chemical moieties in a polymer or copolymer. By this segregation, a fluorine rich Inter-layer between the bulk of the polymer and air is created by the aid of surface tension difference of the fluorinated and organic segments. This behaviour can be enhanced by heat annealing of the polymeric material.

Finally surface topography has a vital effect on wettability and self-cleaning behaviour of the material surface. The phenomenon called "Lotus-Effect" was discovered and published by Barthlott, W. and Neinhus, C., 1997, Purity of the sacred lotus, or escape from contamination in biological surfaces, Planta, 202: 1-8. It was also found that these surfaces are super hydrophobic.

The basis of Lotus effect lies on the presence of many small sized bumps on the solid surface, so when a liquid drop or dirt is attached, the attractive force of the surface is so small that foreign substance cannot stay on it. If the surface is slightly slanted, because of this small contact area the droplets roll off under their own weight and collect the dirt on the tips of bumps and carry them. This is because the attractive force of the water molecules is stronger in total then the surface force, creating a self-cleaning surface.

Applicants' have surprisingly found that also by electro spinning/electro spraying process similar surface roughness and topography can be generated.

In the electro-spinning/ spraying process, a polymer solution or melt, held by surface tension at the end of a capillary, is subjected to a high electric field (Up to 20-30 kV). Charge repulsion causes a force opposite to the surface tension at the tip. As the intensity of the potential field is increased, the surface of the solution at the capillary tip elongates to form a conical shape.

When the electric field reaches a critical value at which repulsive electrical forces overcome surface tension, a jet of the solution is ejected from the tip. This jet is charged and can be directed to a grounded collector.

As the jet travels through the air, the solvent evaporates and this brings thinner fibres. At the end, a continuous, non-woven, ultra-thin (40-2000 nm in diameter) fibres and particles can be collected on the grounded screen.

Electrospraying process needs higher applied voltages than electrospinning. Similar surface roughness as the electrospinning can be created. Instead of nanometer diametered nonwoven fibres, nanometer or micrometer range small, polymer solution droplets are transferred to the grounded screen.

**Table 1. Surface energies and contact angles for water on several substrates.**

| Substrate | Surface Energy | Contact Angle |
|---|---|---|
| PMMA | 41 | 74 |
| Nylon | 38 | 79 |
| Polyethylene | 33 | 96 |
| Polypropylene | 26 | 108 |
| Paraffin | 19 | 110 |
| Teflon | 18 | 112 |
| Clean Glass | 73 | 0 |
| Ordinary Glass | 70 | 20 |

In order that the invention may be more readily understood, reference is made to the following examples which are intended to illustrate the invention, but not restrict or limit whatsoever the scope thereof.

### EXAMPLES

### EXAMPLE 1 - Addition polymerization route with crosslinker

### Materials

In the first reaction scheme:
➢ The meta-Tetramethyl Xylene isocyanate (TMI), also known as Isopropenyl dimethyl benzyl isocyanate, was supplied by Cytec and used in the reactions as received.
➢ The second reactant needed, for the first reaction in the reaction scheme, Acrylo Nitrile (AN), was from Merck (00834) and stabilised with hydroquinone monomethyl ether. Acrylo Nitrile was purified by passing through alumina filled column and dried with anhydrous sodium sulfate before reaction.
➢ For the same reaction, Azoisobutyronitrile (AIBN, Ftuka-11630) was used as initiator and N,N-Dimethyl formamide (DMF, Riedel-15440) was used as solvent. Both were used as receive.

In the second reaction in the reaction scheme,
➢ Fluorolink-D^{®} (a Perfluoropolyether, PFPE, supplied by Ausimont), a diol with 1000 gr/mol average equivalent weight, was used as fluorinated diol HOCH₂CF₂(OCF₂)n(OCF₂CF₂)ₘCF₂CHOH.
➢ Tin (11) 2-ethylhexanoate (T2EH) was supplied from Aldrich (# 28,717-2).
➢ Instead of PFPE, ethylene glycol (Merck # 822329) and
➢ siloxane diol (40 000 gr/mol) containing trials had also been performed.
All chemicals were used as received.

### Synthesis

### 1.Poly (AN-co- TMI)

In a 50ml flask 25ml DMF, 2,51gr TMI, 6,67gr AN and 3mg initiator AIBN are added. Head of the flask is sealed with Aldrich brand Natural Rubber Septa. The solution is shaked for 5 minutes. Than, the content is placed into 70°C oven and kept there for 48 hours for radical polymerisation of monomers in solution. The flask content is stored in -20°C refrigerator when not used.

In order to check the conversion of the reactants to polymer 1,65 gr DMF poly(AN-co-TMI) mixture is added in 15ml methanol and mixed for 10 minutes. The precipitated solid polymer is dried and weighed. The conversion of the reaction is approximately 50-60%.

### 2. a Fluorine containing poly(AN-co-TMI)

1,62gr poly(AN-co-TMI) in DMF is transferred into a separate flask and 0,03gr PFPE is added. To adjust the viscosity to 200-1200 cp range, 1,05gr DMF is also added. After the addition of 3 droplets of T2EH, the content of the flask is mixed for 2 minutes and transferred into glass Pasteur pipettes for electro-spinning purpose.

### 2.b Hydrocarbon containing Poly(AN-co-TMI))

2,09gr poly(AN-co-TMI) In DMF is transferred into a separate flask and 0,06gr Ethylene Glycol is added. To adjust the viscosity to 200-1200 cp range, 0.5340gr DMF is also added. After the addition of 3 droplets of T2EH, the content of the flask is mixed for 2 minutes and transferred into glass Pasteur pipettes for electro-spinning purpose.

### 2_{.}c_{.} Siloxane containing poly(AN-co-TMI

1,18gr poly(AN-co-TMI) in DMF is transferred into a separate flask and 0,27gr siloxane diol is added. To adjust the viscosity to 200-1200 cp range, 1,05gr DMF is also added. After the addition of 3 droplets of T2EH, the content of the flask is mixed for 2 minutes and transferred into glass Pasteur pipettes for electro-spinning purpose.

### Electrospinning

Electrospinning of poly(AN-co-TMI) plus Fluorolink-D^{®} (and Ethylene Glycol and Siloxane diol) mixture is performed, at room temperature conditions, in an apparatus similar as given in Demir MM et al. 2002, Electro-spinning of polyurethane fibres, Polymer. The Pasteur pipette is a glass having 1 mm tip opening, the metal probe is a copper wire that is directly connected to power supply, which is a 50kV CPS Technologies Model 2594.

The grounded collector used was a 20cm x 20cm flat aluminium foil that acted as electrically conductive surface, connected to ground by the aid of a conductive wire. The tip to ground distance was 10 cm. The electro-spinning voltage was 7-20kV.

### Annealing and Casting

After electro-spinning, the aluminium foil was:
a) annealed at 70°C for at least 18 hours under nitrogen atmosphere for complete crosslinking and electrospun, crosslinked and annealed film was obtained.
b) In order to compare the difference between electrospun film and bulk film, the remaining poly(AN-co-TMI) plus PFPE diol mixture is applied over glass lamellas as a thin layer of film and annealed at 70°C. Cast and annealed films are obtained.

### Goniometry Studies

The contact angle measurements of the electrospun and cast films are performed by DSA 10 Mk 2 Goniometry of Krüss GmbH with DSA 1 v.1.7 software.

In the contact angle measurements of the electrospun films on aluminium foil; double-side adhesive coated tape is put onto a glass lamella and the aluminium foil covered with film is cut approximately 10cm² and placed on the adhesive tape.

Contact angle measurements of the electrospun films and cast films on lamellas (with annealing and without annealing) are done without any further treatment. During contact angle measurements, at least six static water droplets, each at the same volume, are studied for the films. The water used for measurements was ultra-pure grade and fresh.

The contact angle (CA) measurements were performed by water and the results are presented at Table 2.

**Table 2. Contact angle measurement results.**

| **Sample** | **Description** | **Water CA(°)** |
|---|---|---|
| Teflon Film | Commercial | 107.20 ± 2.44 |
| Fluorinated 13.3% | Electrospun Web at Figure 3 &4 | 143.20 ± 3.56 |
| Fluorinated 13.3% | Cast film of Figure 3&4 mixture | 88 ± 4.84 |
| Fluorinate 13.3% | Electrospun Web at Figure 2 | 141.45 |
| Fluorinated with 9.3w% Fluorotink-D^{®} | Cast Film - Normal | 102.3 ± 3.39 |
| | Cast Film - Annealed | 106 ± 0.52 |
| | Electrospun - Normal | 149.2 ± 0.85 |
| | Electrospun - Annealed | 154.2 ± 1.62 |
| Ethylene Glycol as diol | Electrospun - Normal | 140.1 ± 1.02 |
| | Electrospun - Annealed | 144.8 ± 0.79 |
| Siloxane diol with 40 000 gr/mol | Electrospun - Normal | 144.9 ± 2.74 |
| | Electrospun - Annealed | 146.6 ± 3.86 |

The measured contact angle values for Teflon are in good agreement with the literature values, which proves the method's applicability. Also, from Table 2, it can be seen that, there ways a huge contact angle value difference between same composition mixture's electrospun-annealed film (154°) and cast film (100°).

### Other Characterisation Instruments

The Scanning electron microscope (SEM) images of poly (AN-co-TMI)+Fluoro-link D at several voltages are presented at Figures 1 to 4. The apparatus used was a Jeol 840A Model Scanning Electron Microscope. For SEM measurement purposes electrospun covered aluminium foils were cut 1cmx1cm. The concentration of the resin mixtures of electrospuns in Figure 2, 3 and 4 were approximately same.

As the spinning voltage decreases, the fibre formation becomes distinct. As the voltage decreases, the attractive force by electrical field is balanced (no excess pull), so stable fibres form from tip to collector and they have found enough time to evaporate solvent.

Also, Applicants have tested if the electrospun product dissolve in DMF or Tetrahydrofuran (THF), the reaction media preferred for the polymerisation reaction. 10ml DMF and 10ml THF are added respectively in 2 flasks and approximately 100mg of electrospun film is added to each flask, that is shaked for 1 hour and left for 1 week. No dissolution of the cured electro-spinning product was observed in either of the reaction media, DMF and THF.

### Effect of Fluorolink-D^{®} Concentration to CA

The optimum value of Fluorolink-D^{®} is important due to economical reasons for industry. So, 1w% to 100w% (relative to solid content in the poly(AN-co-TMI) solution) of Fluorolink-D^{®} are added to the electro-spinning solution.

Also, for each concentration, mixtures are cast filmed on two lamellas. One was annealed, but the other was not to compare the effect of annealing even at cast films. The results are presented at Table 3.

**Table 3. Effect of concentration of Fluorolink-D^{®} to CA.**

| Fluoro-link concentration | 6.4 w% | 9.3w% | 22.5w% | 33.9w% | 56w% | 100w% |
|---|---|---|---|---|---|---|
| Cast Film Annealed | 107.2±5.03 | 106±0.52 | - | 101.9±0.72 | 101.9±1 | 92.8±2.19 |
| Cast Film Normal | 96.4±1.37 | 102.3±3.39 | - | 94.2±2.88 | 103.8±3.95 | 100.1±7.26 |
| E-spun Film Annealed | 146.6±1.92 | 154.2±1.62 | 146.8±2.11 | 142±3.13 | 143.2±1.58 | 143.9±3.88 |

### EXAMPLE 2 - Addition polymerization route without crosslinking reaction

### Materials

The chemicals used are as follows:
➢ Vinyl Benzyl Chloride (VBC) is from Fluka (# 94907),
➢ Dimethylcocoamine is industrial grade,
➢ Sodium carbonate (Na₂CO₃) is supplied from Fluka (#71352)
➢ Perfluoroalkyl ethyl acrylate is Fluowet from Clariant,
➢ Methylmethacrylate (MMA) is from Fluka (# 71351),
➢ AIBN (Fluka-11630) is used as the radical initiator for terpolymer synthesis reaction
➢ THF is Analytical Reagent grade of LabKim.

All chemicals were used as received.

### Synthesis

### Vinyl benzyl-dimethyl cocoammonium chloride (VBDMCAC)

The synthesis of VBDMCAC is carried in a 50 ml round bottom flask. 16.2 gr of dimethylcocamine, 12.6 gr of distilled water and 0.3 gr of Na₂CO₃ is mixed. Than, 8.6 gr of VBC is added while agitating the mixture. The reaction is carried at 50°C under atmospheric pressure and continuous agitation for 2 hours.

### Polymerization for Terpolymer

In a 50ml flask, 1.25 gr perfluoroalkyl ethyl acrylate, 2.23 gr MMA, 0.11 gr VBDMCAC mixture and 0.004 gr AIBN is added into 5.4 gr tetrahydrofuran (THF) solvent. This mixture is degassed for 15 minutes by bubbling with nitrogen gas. The radical polymerization in solution is carried at 70°C for 24 hours. The product is precipitated in 150 ml of industrial grade n-hexane, filtered and dried.

### Electrospinning

Electrospinning is carried in room environment. 0.2 gr of terpolymer is dissolved in 0.5 gr THF and 0.5 gr DMF containing solution. Than the mixture is poured to Pasteur pipette and electrospun with the aid of high voltage generator. The product is collecyed onto 20cmx20cm flat aluminium collector. The tip to ground distance is 10 cm and the electrospinning voltage is 12 kV.

### Goniometry Study

The contact-angle measurement of the electrospun film is performed by DSA 10 Mk 2 Goniometry of Krüss GmbH with DSA 1 v.1.7 software. Not annealed was 159.2±2.4.

In the contact angle measurements of the electrospun films on aluminium foil; double-side adhesive coated tape is put onto a glass lamella and the aluminium foil covered with film is cut approximately 10cm² and placed on the adhesive tape. During contact angle measurements, at least six static water droplets, each at the same volume, are studied for the films. The water used for measurements was ultra-pure grade and fresh.

### EXAMPLE 3 - Condensation polymerization route

### Materials

The chemicals used are as follows:
➢ HO-R_{H}-OH is Polyethylene Glycol (PEG 4000) with a molecular weight of 4000 gr/mol from Merck (# 07490),
➢ Methylene diphenyl diisocyanate (MDI, C₁₅H₁₀N₂O₂) is from Acros (# 41428),
➢ Tin (II) 2-ethylhexanoate (T2EH) is supplied from Aldrich (# 28,717-2),
➢ Dimethylol butanoic acid (DMBA, C₆H₁₂O₄) is from Marubeni Corporation,
➢ R_{F}-OH is perfluoroalkyl ethanol (PFAE, Fluowet^{®} EA 600) from Clariant,
➢ Thionyl chloride is from Merck (# 808154) and
➢ Pyridine is from LabScan (# G4544).

All chemicals were used as received.

### Synthesis

### Prepolymer A

In a 50ml round bottom flask, 30ml toluene solvent, 1gr MDI and 8gr PEG 4000 are added. 6-7 droplets of T2EH are also added to the flask as reaction catalyst. During the reaction, the head of the flask is covered with Rubber Septa, the mixture is agitated and kept under nitrogen atmosphere. The reaction is carried out for 24 hours at room temperature.

### Prepolymer B

Prepolymer B is synthesized in two steps. First, in a 50ml flask 7.4 gr of DMBA is refluxed with 30 ml Thionyl Chloride overnight and than, the chlorinated DMBA is purified by evaporation. In the second step, 3.33gr of chlorinated DMBA is reacted with 7.4gr of Fluowet^{®} (PFAE) in 30ml Toluene. As acid scavenger 6-7 drops of pyridine is added and the reaction is carried for 3 hours at room temperature. The product is filtered to remove Pyridine.HCl complex and Prepolymer B solution.

### Polymerization

The required amount of Prepolymer A and Prepolymer B solutions for polymerization is calculated by determination of reactive groups with the titration method. In a 50ml flask, Prepolymer A solution (29.3m1) and Prepolymer B solution (2.28ml) are mixed. As catalyst 8-9 droplets of T2EH is added. The reaction is carried at 80°C for 48 hours. After the reaction is complete, the reaction mixture is poured into 300ml of n-hexane and the product is precipitated. The precipitate is filtered with filter paper and dried in vacuum oven at room temperature for 48 hours.

### Electrospinning

Electrospinning of polycondensation reaction product is carried at room temperature. 0.5 gr of condensation polymer is dissolved in 2.1 ml of DMF. Than the mixture is poured to Pasteur pipette and electrospun with the aid of high voltage generator. The product is collected on the grounded collector.

The grounded collector used is a 20cm x 20cm flat aluminium foil that acted as electrically conductive surface, connected to ground by the aid of a conductive wire. The tip to ground distance was 15 cm. The electro-spinning voltage was 8-15kV.

### Annealing

After electro-spinning, the aluminium foil was annealed at 70°C for at least 18 hours under nitrogen atmosphere for complete crosslinking. An electrospun, crosslinked and annealed film was obtained.

### Goniometry Studies

The contact-angle measurement of the electrospun film is performed by DSA 10 Mk 2 Goniometry of Krüss GmbH with DSA 1 v.1.7 software.

In the contact angle measurements of the electrospun films on aluminium foil; double-side adhesive coated tape is put onto a glass lamella and the aluminium foil covered with film is cut approximately 10cm² and placed on the adhesive tape.

### INDUSTRIAL APPLICATION

This physical phenomenon is an important property of materials mostly at printing industry, painting industry, membrane-manufacturing industry, lubricant industry or textile industry. So, determination and regulation of this physical property is crucial for the performance of many materials in their application fields.

Some implantation areas of super-hydrophobic surfaces are for example the prevention of adhesion of dirt and foreign materials to the materials. It can be used in antennas, bio-reactors, solar cells, traffic indicators, public transports, animal cages, etc.

One other application may be stain resistance of the materials. It can be used in saunas, swimming-pools, bathrooms, kitchens, roofs, walls, facades, green-houses, garden fences, wood appliances, etc.

One further application may be against the sticking of marine organisms and plants to the marine constructions, because if even the water cannot wet the surface, how can the marine organisms can stick on it. Antifouling applications may be used in human made marine vessels and buildings, haven appliances, oil-drilling platforms, etc.

Other application areas of electrospun fibres are multi-functional membranes, biomedical structural elements (scaffolding used in tissue engineering, wound dressing, drug delivery, artificial organs), protective shields in specialty fabrics, filter media for submicron particles in separation industry, composite reinforcement, and structures for nano-electric machines.

The terms and expressions which have been employed are used as terms of description and not of limitations, and there is no intention in the use of such terms or expressions of excluding any equivalents of the features shown and described as portions thereof. It will be obvious to those skilled in the art that various changes may be made without departing from the scope of the invention which is not be considered limited to what is described in the specification.

## Claims

1. A process for preparing super hydrophobic surface compositions comprising the steps
a) radical or condensation polymerisation of a reactive functional group containing monomer pair with an initiator in non-reactive solvent environment, and
b) mixing the copolymer obtained in a) with a hydrocarbon/fluorinated/siloxane chemical agent having at least one end capped with reactive groups and a catalyst.
**characterised in that** it further comprises the step of
c) electrospinning/ electrospraying of the mixture obtained in b), and
d) annealing and crosslinking of the electrospun/ electrosprayed mixture.

2. Process according to claim 1 **characterised In** step a) that the monomer pairs are radical or condensation polymerisable monomers and their combination and step growth polymerisable monomers where one of them contains fluoro/siloxane/hydrocarbon alkyl group and a reactive functional group chosen from the group comprising TMI/AN, TMI/Styrene, TMI/polymethylmethacrylate, and perfluoro-alkyl acrylate/vinyl benzyl-dimethyl-cocoamonium chloride (VBDMCAC).

3. Process according to any one of the preceding claims, **characterised in that** in step a) the inert environment is a non reactive solvent chosen from the group comprising dimethyl formamide (DMF), tetrahydro furane (THF), chloroform, methylene chloride, toluene, dichloromethane, ethanol, formic acid, dimethylacetamide, acetone.

4. Process according to any one of the preceding claims, **characterised in that** in step a) the initiator is a radical generating initiator or condensation polymerisation catalyst chosen from the group comprising azo initiators, peroxide initiators, ammonium persulphate, sodium persulphate and stannous-2-ethyl hexanoate (T2EH), cobalt-2-ethyl hexanoate, dibutyltin dilaurate.

5. Process according to any one of the preceding claims, **characterised in that** in step b) the hydrocarbon/fluorinated/siloxane chemical agent having both ends capped with reactive groups such as hydroxyl, amine, carboxyl, isocyanate and thiol is a diol containing agent chosen between fluorinated diols, siloxane diols and hydrocarbon diols, preferably chosen from the group comprising (perfluoropolyether, PFPE) HOCH₂CF₂(OCF₂)ₙ(OCF₂CF₂)ₘCF₂CH₂OH, (siloxane diols) HO(Me₂Si-O)ₙH, (hydrocarbon diol) HO(CH₂)ₙOH, and (polyether diol) HO(CH₂CH₂O)ₙH.

6. Process according to any one of the preceding claims, **characterised in that** in step b) the catalyst is chosen from organometallic catalysts comprising stannous-2-ethyl hexanoate (T2EH), cobalt-2-ethyl hexanoate, dibutyltin dilaurate.

7. Process according to any one of the preceding claims, **characterised in that** in step c) the mixtures are electrospun/sprayed at 5-35 kV and 5-25 cm tip distance.

8. Process according to any one of the preceding claims, **characterised in that** in step d) the electrospun/sprayed mats are annealed above the glass transition temperature.

9. Super-hydrophobic surface compositions obtained by a process according to any one of the preceding claims, **characterised in that** their water contact-angle at least 140°.

10. Use of the super-hydrophobic surface compositions according to claim 9 In the prevention of adhesion of dirt and foreign materials to materials like antennas, windows, bio-reactors, solar cells, traffic indicators, public transports and animal cages.

11. Use of the super-hydrophobic surface compositions according to claim 9 in antifouling applications in human made marine vessels and buildings, haven appliances and oil-drilling platforms.

12. Use of the super-hydrophobic surface compositions according to claim 9 in stain resistance of the materials in saunas, swimming-pools, bathrooms, kitchens, roofs, walls, facades, green-houses, garden fences, wood appliances.

13. Use of the super-hydrophobic surface compositions according to claim 9 in multi-functional membranes, biomedical structural elements (scaffolding used in tissue engineering, wound dressing, drug delivery, artificial organs), protective shields in specialty fabrics, filter media for submicron particles in separation industry, composite reinforcement, and structures for nano-electric machines.

## Patentansprüche

1. Verfahren zum Herstellen von super-hydrophoben Oberflächenzusammensetzungen, umfassend die Schritte:
a) Radikalpolymerisation oder Kondensationspolymerisation einer reaktiven funktionellen Gruppe, die ein Monomerpaar enthält, mit einem Initiator in nicht-reaktiver Lösungsmittelumgebung, und
b) Mischen des in a) erhaltenen Copolymers mit einem chemischen Kohlenwasserstoffmittel/fluorierten chemischen Mittel/chemischen Siloxanmittel, das zumindest ein mit reaktiven Gruppen gecapptes Ende aufweist, und mit einem Katalysator,
**dadurch gekennzeichnet, dass** es weiters den Schritt umfasst:
c) Elektrospinnen/Elektrosprühen der in b) erhaltenen Mischung, und
d) Anlassen und Vernetzen der elektrogespinnten/elektrogesprühten Mischung.

2. Verfahren nach Anspruch 1, **dadurch gekennzeichnet, dass** in Schritt a) die Monomerpaare radikalisch polymerisierbare oder kondensationspolymerisierbare Monomere und ihre Kombination und stufenwachstumspolymerisierbare Monomere sind, wobei eines von diesen eine Fluor-/Siloxan-/Kohlenwasserstoff-Alkylgruppe und eine reaktive funktionelle Gruppe, ausgewählt aus der Gruppe umfassend TMI/AN, TMI/Styrol, TMI/Polymethylmethacrylat und Perfluoralkylacrylat/Vinylbenzyldimethylcocoammonium (VBDMCAC), enthält.

3. Verfahren nach einem der vorhergehenden Ansprüche, **dadurch gekennzeichnet, dass** in Schritt a) die inerte Umgebung ein nicht-reaktives Lösungsmittel ist, das aus der Gruppe umfassend Dimethylformamid (DMF), Tetrahydrofuran (THF), Chloroform, Methylenchlorid, Toluen, Dichlormethan, Ethanol, Ameisensäure, Dimethylacetamid, Aceton ausgewählt ist.

4. Verfahren nach einem der vorhergehenden Ansprüche, **dadurch gekennzeichnet, dass** in Schritt a) der Initiator ein radikalbildender Initiator oder ein Kondensationspolymerisationskatalysator, ausgewählt aus der Gruppe umfassend AzoInitiatoren, Peroxid-Initiatoren, Ammoniumpersulfat, Natriumpersulfat und Zinn-2-ethylhexanoat (T2EH), Kobalt-2-ethylhexanoat, Dibutylzinndilaureat, ist.

5. Verfahren nach einem der vorhergehenden Ansprüche, **dadurch gekennzeichnet, dass** in Schritt b) das chemische Kohlenwasserstoff-/fluorierte/Siloxan-Mittel, bei dem beide Enden mit reaktiven Gruppen, beispielsweise Hydroxyl, Amin, Carboxyl, Isocyanat und Thiol, verschlossen sind, ein diolhältiges Mittel ist, das aus fluorierten Diolen, Siloxandiolen und Kohlenwasserstoffdiolen, vorzugsweise aus der Gruppe umfassend (Perfluorpolyether, PFPE) HOCH₂CF₂(OCF₂)ₙ(OCF₂CF₂)ₘCF₂CH₂OH, (Siloxandiole) HO(ME₂Si-O)ₙH, (Kohlenwasserstoffdiol) HO(CH₂)ₙOH, und (Polyetherdiol) HO(CH₂CH₂O)ₙH), ausgewählt ist.

6. Verfahren nach einem der vorhergehenden Ansprüche, **dadurch gekennzeichnet, dass** in Schritt b) der Katalysator aus organometallischen Katalysatoren ausgewählt ist, die Zinn-2-ethylhexanoat (T2EH), Kobalt-2-ethylhexanoat, Dibutylzinndilaureat umfassen.

7. Verfahren nach einem der vorhergehenden Ansprüche, **dadurch gekennzeichnet, dass** in Schritt c) die Mischungen bei 5 bis 35 kV und einem Abstand der Spitzen von 5 bis 25 cm elektrogespinnt/elektrogesprüht werden.

8. Verfahren nach einem der vorhergehenden Ansprüche, **dadurch gekennzeichnet, dass** in Schritt d) die elektrogespinnten/elektrogesprühten Matten über Glasübergangstemperatur aufgeschmolzen werden.

9. Super-hydrophobe Oberflächenzusammensetzungen, die mit einem Verfahren anch einem der vorhergehenden Ansprüche erhalten wurden, **dadurch gekennzeichnet, dass** ihr Wasserkontaktwinkel zumindest 140° beträgt.

10. Verwendung der super-hydrophoben Oberflächenzusammensetzungen nach Anspruch 9 bei der Prävention von Schmutz- und Fremdmaterialanhaftung an Materialien wie Antennen, Fenster, Bioreaktoren, Solarzellen, Verkehrsanzeigevorrichtungen, öffentliche Verkehrsmittel und Tierkäfigen.

11. Verwendung der super-hydrophoben Oberflächenzusammensetzungen nach Anspruch 9 bei fäulnisverhütenden Anwendungen in von Menschen gebauten Seefahrzeugen und Gebäuden, Hafeneinrichtungen und Ölbohrinseln.

12. Verwendung der super-hydrophoben Oberflächenzusammensetzungen nach Anspruch 9 bei der Fleckenbeständigkeit von Materialien bei Saunen, Schwimmbecken, Bädern, Küchen, Dächern, Wänden, Fassaden, Gewächshäusern, Gartenzäunen, Holzeinrichtungen.

13. Verwendung der super-hydrophoben Oberflächenzusammensetzungen nach Anspruch 9 bei multifunktionellen Membranen, biomedizinischen Bauelementen (Gerüst, das bei der Gewebezüchtung, bei Wundverbänden, der Arzneimittelzufuhr, künstlichen Organen verwendet wird), Schutzschilden in Fachfabriken, Filtermedien für Submikron-Partikel in der Trennungsindustrie ("separation industry"), Verbundverstärkung und Strukturen für nanoelektrische Maschinen.

## Revendications

1. Procédé de préparation de compositions de surface super-hydrophobes comprenant les étapes de
a) polymérisation radicalaire ou de condensation d'un groupe fonctionnel réactif contenant une paire de monomères avec un initiateur dans un environnement de solvant non réactif, et
b) mélange du copolymère obtenu dans a) avec un agent chimique hydrocarbure/fluoré/siloxane ayant au moins une extrémité coiffée par des groupes réactifs et un catalyseur,
**caractérisé en ce qu'**il comprend en outre les étapes de
c) électrofilage/électropulvérisation du mélange obtenu en b), et
d) recuit et réticulation du mélange électrofilé/électropulvérisé.

2. Procédé selon la revendication 1, **caractérisé en ce que** dans l'étape a), les paires de monomères sont des monomères polymérisables par radicaux ou condensation et leur combinaison et des monomères polymérisables par croissance par palier où l'un d'entre eux contient un groupe alkyl fluoro/siloxane/hydrocarbure et un groupe fonctionnel réactif choisi dans le groupe comprenant TMI/AN, TMI/styrène, TMI/poly(méthacrylate de méthyle) et perfluoro-acrylate d'alkyle/chlorure de vinyl benzyl-diméthyl-cocoammonium (VBDMCAC).

3. Procédé selon l'une quelconque des revendications précédentes, **caractérisé en ce que** dans l'étape a), l'environnement inerte est un solvant non réactif choisi dans le groupe comprenant le diméthylformamide (DMF), le tétrahydrofurane (THF), le chloroforme, le chlorure de méthylène, le toluène, le dichlorométhane, l'éthanol, l'acide formique, le diméthylacétamide et l'acétone.

4. Procédé selon l'une quelconque des revendications précédentes, **caractérisé en ce que** dans l'étape a), l'initiateur est un initiateur générant des radicaux ou un catalyseur de polymérisation par condensation choisi dans le groupe comprenant les initiateurs azoïques, les initiateurs peroxydes, le persulfate d'ammonium, le persulfate de sodium et le 2-éthyl hexanoate stanneux (T2EH), le 2-éthyl hexanoate de cobalt et le dilaurate de dibutylétain.

5. Procédé selon l'une quelconque des revendications précédentes, **caractérisé en ce que** dans l'étape b), l'agent chimique hydrocarbure/fluoré/siloxane ayant les deux extrémités coiffées par des groupes réactifs tels qu'hydroxyde, amine, carboxyle, isocyanate et thiol est un agent contenant un diol choisi parmi les diols fluorés, les siloxane diols et les hydrocarbure diols, de préférence choisi dans le groupe comprenant (perfluoropolyéther, PFPE) HOCH₂CF₂(OCF₂)-ₙ(OCF₂CF₂)ₘCF₂CH₂OH, (siloxane diols) HO(Me₂Si-O)ₙH, (hydrocarbure diol) HO(CH₂)ₙOH et (polyéther diol) HO(CH₂CH₂O)ₙH.

6. Procédé selon l'une quelconque des revendications précédentes, **caractérisé en ce que** dans l'étape b), le catalyseur est choisi parmi les catalyseurs organométalliques comprenant le 2-éthyl hexanoate stanneux (T2EH), le 2-éthyl hexanoate de cobalt et le dilaurate de dibutylétain.

7. Procédé selon l'une quelconque des revendications précédentes, **caractérisé en ce que** dans l'étape c), les mélanges sont électrofilés/pulvérisés à 5 à 35 kV et une distance d'embout de 5 à 25 cm.

8. Procédé selon l'une quelconque des revendications précédentes, **caractérisé en ce que** dans l'étape d), les matelas électrofilés/pulvérisés sont recuits au-delà de la température de transition vitreuse.

9. Compositions de surface super-hydrophobes obtenues par un procédé selon l'une quelconque des revendications précédentes, **caractérisées en ce que** leur angle de contact avec l'eau est d'au moins 140°.

10. Utilisation des compositions de surface super-hydrophobes selon la revendication 9, dans la prévention de l'adhérence de saleté et de matières étrangères sur des matériaux comme des antennes, des fenêtres, des bioréacteurs, des piles solaires, des indicateurs de trafic, des transports publics et des cages pour animaux.

11. Utilisation des compositions de surface super-hydrophobes selon la revendication 9, dans des applications anti-salissures dans des vaisseaux marins et des constructions fabriqués par l'homme, les instruments de port marin et les plateformes de forage de pétrole.

12. Utilisation des compositions de surface super-hydrophobes selon la revendication 9, dans la résistance aux taches des matériaux dans des saunas, piscines, salles de bains, cuisines, toits, murs, façades, serres, clôtures de jardin et instruments en bois.

13. Utilisation des compositions de surface super-hydrophobes selon la revendication 9, dans des membranes multifonctiennelles, des éléments structurels biomédicaux (échafaudage utilisé dans l'ingénierie tissulaire, les pansements, l'administration de médicament, les organes artificiels), des blindages protecteurs dans des tissus de spécialité, des milieux filtrants pour des particules submicrométriques dans l'industrie de la séparation, le renforcement des composites, et les structures pour des machines nano-électriques.
